

[72] Inventor **Robert Cone**  
599 River Road, Piermont, N.Y. 10968  
[21] Appl. No. **804,046**  
[22] Filed **Feb. 10, 1969**  
[45] Patented **Oct. 26, 1971**

[54] **HIGH-SPEED PHOTOGRAPHIC EMULSION AND  
METHOD OF USING SAME**  
2 Claims, No Drawings

[52] U.S. Cl..... **96/36.4**  
[51] Int. Cl..... **G03c 5/00**  
[50] Field of Search..... **96/36.4, 94,  
114.7**

[56] **References Cited**

UNITED STATES PATENTS

|           |         |              |          |
|-----------|---------|--------------|----------|
| 2,694,637 | 11/1954 | Gray.....    | 96/114.7 |
| 2,969,014 | 1/1961  | Hanson ..... | 96/36.4  |
| 3,458,317 | 7/1969  | Ditzer.....  | 96/94    |

OTHER REFERENCES

"Photographic Chemistry," Pierre Glafkides, pp. 375, 380,  
381, 382, 383 (1957)  
Primary Examiner—Norman G. Torchin  
Assistant Examiner—Judson R. Hightower  
Attorney—Charles E. Temko

**ABSTRACT:** A projection-speed silver bromide emulsion of washed type and containing by weight of the silver nitrate used in making the emulsion of an organic antifoggant in excess of 1.5 percent, a retarder consisting of a crystalline quaternary ammonium salt such as di-isobutyl phenoxy (or cresoxy) ethoxy ethyl dimethyl benzyl ammonium chloride monohydrate of approximately 0.1 percent (which also serves as a germicide), and a hardener ranging between 0.04 and 0.15 of the total weight of the gelatin in the emulsion.

## HIGH-SPEED PHOTOGRAPHIC EMULSION AND METHOD OF USING SAME

This invention relates generally to the field of silk screen photographic emulsions, and more particularly to an improved emulsion of enlargement speed, permitting the use of a stencil material coated with such emulsion directly in the copy camera.

In the making of silk screen stencils by photographic methods, the usual process employs contact speed emulsions of dichromate type, necessitating the making of a film positive in the same size as the screen. The film positive is then placed over the screen and a brilliant light source is used to directly harden the emulsion in the areas where the light penetrates the film.

In accordance with my invention, and the process using it, a coated screen may be placed directly in the process camera where the film would ordinarily be placed in conventional methods. The screen then registers the image directly from the original art work, following which the screen is given a developer bath with a sponge and washed out in warm water. The result is a screen that is a negative stencil of the original art work, and can be used for printing purposes. An alternative method of silk screen making utilizing a projection speed emulsion entails the use of a small film positive in an enlarger. The film positive is therefore projected onto the screen, enabling large silk screens to be made with small film positives. The significance of improved speeds in such an emulsion is that a totally different method of processing can be obtained, one that eliminates a great deal of time and effort. This is an obvious advantage in economy as well as time, since traditional methods dictate the use of a large film positive and a vacuum frame, in addition to large lighting equipment to make contact process screens.

It is therefore among the principal objects of the present invention to provide an improved high speed silver bromide emulsion, whereby the direct exposure of the sensitized silk screen to art copy is possible.

Another object of the invention lies in the provision of an improved method utilizing the above high-speed emulsion, with consequent substantial savings in time and expense.

These objects, as well as other incidental ends and advantages, will more fully appear in the progress of the following disclosure, and be pointed out in the appended claims.

Briefly stated, the invention contemplates the making of a silver bromide emulsion in a gelatin suspension. The emulsion is preferably washed, that is to say, it contains little or no potassium nitrate as a result of rinsing away by water. The resultant pure silver bromide emulsion is of a type which is commonly used for black and white film, and also for coating fast enlargement papers. The bromide emulsion is coated on the silk screen, and after exposure the screen is rinsed with a developing solution containing pyrogallol and metol, plus a base. The purpose of the development is to both reduce the latent image to pure silver, and also to tan the gelatin locally in the pure silver area. Pyrogallol is one of the developers which has the capacity of tanning the gelatin in the presence of pure silver. Other well-known developers such as hydroquinone and pyrocatechin may also be used, however. The portions of the emulsion that have been tanned by the developer thus become insoluble, due to the tanning of the gelatin. When the screen is placed in warm water, the gelatin which has not been tanned washes away, leaving the hardened gelatin. Thus, it may be observed that the developer acts simultaneously to reduce the light-activated silver bromide to metallic silver, and tan the gelatin locally in the presence of reduced silver.

In the above described process, the substitution of a high-speed silver bromide emulsion for the more traditional dichromate emulsion is not without substantial modification of conventional silver bromide type of emulsions. Traditionally, the contact speed emulsions have been employed in the silk screen process for the reason that such emulsions possess substantially superior contrast characteristics which facilitates the tanning action and subsequent removal of unwanted gelatin. So that the contrast qualities of the silver bromide emulsion

employed are adequate for the present purpose, after washing to increase speed, substantial quantities of restrainer and organic antifog are added to the emulsion. Certain quaternary ammonium salts make an excellent restrainer, and is required to exceed approximately 0.1 percent by weight of the silver nitrate used in making the emulsion. The amount of organic antifog, preferably benzotriazol must exceed 1.5 percent the total weight of silver nitrate used in making the emulsion, the preferred range being from 1.5 percent to 2.0 percent. For different restrainers and/or antifogs, different percentages would apply. In each case, however, the quantities required are substantially greater than those of conventional high-speed photographic emulsions.

A second distinctive characteristic of the emulsion is the presence of a hardener in the finished emulsion. The hardener must not be present in such great quantity as to insolubilize the gelatin, as is the case with hardeners that are added before emulsions are coated on paper or film, but sufficient to substantially aid the tanning process encountered on developing after exposure. In the case of potassium chrome alum, when used as the sole hardener in the emulsion, the proportion should not be less than 0.4 percent and should not exceed 0.15 percent of the total weight of gelatin in the emulsion. The reason for this critical factor is that the tanning developers which are used, e.g., pyrogallol with metol, are not sufficiently powerful to provide sufficient tanning of an emulsion without some hardener. However, a hardener in quantities above that indicated would hamper clean and easy washout of the screen and would, in a sufficient quantity, cause the emulsion eventually to be difficult to liquify at the temperatures which would be harmless to the emulsion by considerably raising the melting point of the gelatin beyond a practical range. Further, the gelatin content of the emulsion must be greater than that used for paper or film, in the order of at least 200 grams of gelatin per liter of the emulsion. If substantially less gelatin is used, the emulsion will be difficult to coat as it will flow through the screen, and if substantially greater quantities are used, the tanning action will be impaired. In summary, therefore, it is possible to attribute certain distinctive characteristics to the emulsion. It is a washed emulsion, predominately bromide, with an unusually large amount of restrainer and/or antifog added for contrast, and long shelf life, a critical amount of hardener, and a relatively high-gelatin content. A side benefit of the large amount of restrainer plus antifog is that the emulsion demonstrates unusually good storage properties, and can generally be kept for as long as 3 months at normal room temperatures. This is due to the fog restraining activity of these types of compounds. The emulsions may, if desired, contain other additives, as do most photographic emulsions, such as plasticizers and surface active agents to achieve greater ease of handling.

My process also lends itself to the production of reversed reliefs. As is known in the art, not only can gelatin be tanned locally in the presence of silver, but it may also be softened locally in the presence of silver. This is customarily achieved in the art through the use of hydrogen peroxide. Positive art work may thus be used to produce a positive screen. This aspect of the invention may be applied to screen making on a practical basis by using a film negative to project line or half-tone art work onto a screen to achieve a negative screen. Let us assume that a photographic amateur using ordinary film is interested in making silk screens. He may then photograph original art work (positive) using a conventional panchromatic film. The negative may then be placed in an enlarger, and a screen coated with the disclosed emulsion placed under the enlarger prior to making exposure. Using the reverse relief process above described, he may then produce a negative screen corresponding to the reverse of the original art work. This negative screen is then used for printing purposes to produce a final positive print when inked. Thus, through reversal processing coupled with the use of this emulsion, a vastly wider range of silk screen processes may be created. Note, that without reversal processing, the amateur would

have to obtain a film positive of the original art work, assuming that he commenced with positive art work, before placing it in the enlarger in order to obtain a negative screen. Thus, reversal processing coupled with the use of an enlargement speed emulsion are both necessary to provide silk screen benefits to a much wider audience than is available in the case of contact printing methods. Reversal processing is achieved through the conventional use of hydrogen peroxide (plus a halogenizing agent, in this case cupric chloride in an acid solution) suggests another important application area for my emulsion, which is the making of photoengraving plates directly with a camera, and without intermediate steps connected with film making. The photoengraver simply coats a metal plate with emulsion, and places it in the process camera where the film would ordinarily be located. He then photographs the original art work (positive) onto the sensitized plate, using the reversal processing technique to make a positive photoresist plate. The emulsion areas on the plate after processing will correspond to the unexposed portions of the emulsion. The coated plate may then be hardened either chemically or through the use of moderate heat in order to withstand the etchant solution. The use of pure gelatin as the colloidal agent will not, of course, provide as great a degree of resistance to etching as will other so-called enamels that are used as conventional engraving resists. However, gelatin does offer a degree of resistance satisfactory for many needs, and if necessary, limited amounts of other colloids, such as fish glue, may be added to the emulsion in order to increase adhesion to the plate and resistance to the etching solution. Correspondingly, a greater amount of hardener must be incorporated into the emulsion used for plate making purposes than is the case in the making of silk screen emulsions, in order to overcome the tendency of the emulsion to lack adhesion to a smooth metal surface. However, the proportion of hardener assuming the use of chrome alum should still not be so great as to prevent liquification of the emulsion at a temperature of 120° F. or less, which is the maximum for practical purposes of shelf life.

The techniques described here and above for silk screen or photoengraving use may also be applied with suitable modification through a wide range of graphic applications. Many printing processes such as collotype, offset, intaglio, etc. require the use of a photosensitive emulsion. The purpose may be to provide a relief surface, or to form a surface that attracts or repels greasy or water-base inks. The latter described procedure is the basis for the familiar photo offset printing process. In all of these cases, the basic emulsion described herein is an appropriate agent.

The following examples are illustrative, and are given as specific examples of exact methods of carrying out the invention. It will be understood that modifications within the scope of the invention are possible by those skilled in the art to which the invention pertains.

#### EXAMPLE 1

A silver bromide emulsion is made by conventional methods using silver nitrate and potassium bromate, washing the same to remove substantially all traces of potassium nitrate. To this emulsion, an organic antifog agent benzotriazol is added, ranging from 1.5 percent to 2.0 percent by weight of the silver nitrate ordinarily used, followed by approximately 0.1 percent of a retarder and organic antifog agent, di-isobutyl phenoxy (or cresoxy) ethoxy ethyl dimethyl benzyl ammonium chloride monohydrate, similarly computed, and 0.04 percent to 0.15

percent of potassium chrome alum based on the weight of gelatin in the emulsion.

The above admixture is combined with relatively hard gelatin in the proportions of approximately 200 grams of gelatin per liter of emulsion, following which it is ready to be applied to conventional silk screen stencil material.

Coating may be accomplished in conventional manner, using spraying, dipping, or doctor blade techniques, all of which are known in the art, following which the emulsion is permitted to cool and harden.

In the above described proportions of emulsion and gelatin, the prepared suspension will have an ASA rating approximately the same as fast process film, permitting it to be directly exposed in a copy camera with relatively short exposure time.

The developing and tanning process is best performed with a sponge dipped in the developing solution, and following the reduction to metallic silver and subsequent tanning of the exposed portions of the gelatin, the remaining soft gelatin is gently flushed away with warm water. The developing solution is a conventional metol-pyrogallol type well-known in the art, or in the alternative, a metol-hydroquinone developer may also be employed. As the hardener is incorporated directly in the emulsion, no separate hardening and bleaching step is necessary, and after drying, the stencil is ready for immediate use.

#### EXAMPLE 2

A silver bromide emulsion is prepared as in Example 1, and coated upon the stencil and exposed as in that example. After developing the exposed emulsion with conventional (non-tanning) paper developer, the stencil is subjected to the action of a mild acid solution of hydrogen peroxide and cupric chloride, which results in the softening of the exposed areas of the gelatin relative to the unexposed areas. In this case, the potassium chrome alum present in the emulsion will sufficiently harden the unexposed areas of the exposed image to permit a reverse relief.

I wish it to be understood that I do not consider the invention limited to the precise details of structure shown and set forth in this specification, for obvious modifications will occur to those skilled in the art to which the invention pertains.

I claim:

1. The method of preparing a silk screen stencil photographically, including the steps of: preparing a high-speed silver bromide emulsion, washing said emulsion to substantially remove any potassium nitrate present, mixing said emulsion with a relatively hard gelatin to form a suspension in the ratio of at least 200 grams of gelatin per liter of emulsion, adding 0.04 percent to 0.15 percent of potassium chrome alum, approximately 1.5 percent benzotriazol, and approximately 0.1 percent of a quaternary ammonium salt, each by weight of the amount of silver nitrate used; coating a porous stencil screen with said suspension to block the mesh thereof, exposing said screen to a projected light image, subjecting the exposed screen to the action of a tanning developer selected from the group consisting of pyrogallol, hydroquinone and pyrocatechin, wherein exposed portions of the emulsion become insoluble, and subsequently subjecting the developed screen stencil to the action of warm water whereby untanned gelatin is washed away.

2. The method in accordance with claim 1, including the step of subjecting the exposed and developed image to the action of a gelatin-softening agent, including hydrogen peroxide.

\* \* \* \* \*

65

70

75